

## UNITED STATES PATENT OFFICE

2,083,013

## METAL CLEANER

Michael W. Freeman, Detroit, Mich.

No Drawing. Application February 15, 1932, Serial No. 593,208. Renewed February 17, 1934

5 Claims. (Cl. 148—8)

The present invention relates to the cleaning of metals and more particularly to the preparation of iron and steel surfaces to be subsequently coated with a protective film. The invention will be described in connection with steel, but it is in no way limited to that particular metal.

Metal cleaners are used in many arts, and such cleaners are widely used in the manufacture of automobile bodies and metal furniture. In the making of such articles, the metals are usually pickled, shaped, and joined together to give the desired structure. During the forming and joining of the metal pieces, the metal surfaces become soiled with handling marks, greases of various natures, and the like, and also become corroded so that it is essential that such foreign matter contained on the surface of the metal be removed before coating thereof with protective films such as by painting, lacquering, metallic plating, and the like.

In the past, it is my understanding that cleaners, including a mineral acid or mixture of mineral acids, have been used for removing the foreign material from such metal surfaces. The most customary mineral acid employed has been phosphoric acid and/or various salts thereof. In the use of these prior art cleaning mixtures, including the mineral acid, the metal surfaces have first been washed to remove excess of oil and grease, such solvents as commercial gasoline being employed for this purpose.

Subsequent to the washing in this manner, the cleaner has been applied to the metal and, because of the ingredients used in the prior art cleaners, it has not been feasible to spray the same upon the metal due to the obnoxious acid fumes resulting from the spraying. By reason of the inability to spray the cleaner, it has been necessary to apply the same by means of cloths, brushes, and such equipment.

Obviously, due to the presence of the mineral acid in the cleaning fluid, it is essential that the cleanser be thoroughly washed from the metal to prevent further corrosion. This washing may be accomplished by the use of hot water to get rid of the free acid or, in lieu of water, a weak base such as ammonium hydroxide can be used as a neutralizing agent.

After washing, the metal surfaces are dried and then painted or otherwise provided with the protective coating.

Because of the use of the mineral acid cleaner, in most cases the metal surface has an undesirable dark film left thereon. The thorough dry-

ing of the cleaned metal prior to painting is of prime importance to the prior art processes.

It is an important object of the present invention to provide a cleaning compound for metallic surfaces including an organic sulphonlic acid, mixtures or derivatives thereof, dissolved in a suitable solvent or mixture of solvents.

Another important object of the invention is to provide such a cleaner which is substantially, if not entirely, devoid of mineral acids so that after application of the cleaning material, it is not essential to the successful operation to remove said cleaning material from the metal surface.

There are numerous other objects of the invention that will become apparent hereinafter.

Broadly speaking, I produce my improved metal cleaner by making a mixture of an organic sulphonlic acid, a solvent therefor, and a solvent for grease. The invention contemplates the use of any organic sulphonlic acid which includes sulphonlic acids of the aromatic or aliphatic hydrocarbons or derivatives thereof. Examples of these sulphonlic acids are: Phenol sulphonlic acid; benzene sulphonlic acid; naphthalene sulphonlic acid; toluene sulphonlic acid; naphthol sulphonlic acid, and others.

Obviously, the exact proportions of any mixture will depend upon the particular organic sulphonlic acid used as well as the solvents included. In addition, the particular character of metallic surface to be cleaned must be taken into consideration. However, by way of example, I will point out that the following mixture has been commercially used in the cleaning of automobile bodies in a very satisfactory manner:

|                                   | Percent |
|-----------------------------------|---------|
| Crude naphthalene sulphonlic acid | 6       |
| Denatured alcohol                 | 50      |
| Water                             | 34      |
| Benzene                           | 10      |
|                                   | 40      |

In this particular mixture, the water serves as a solvent for the crude naphthalene sulphonlic acid, while the alcohol and benzene are primarily included for dissolving the grease on the metal so that the sulphonlic acid solution will penetrate readily to the surface of the metal being treated. The alcohol and benzene also, in the example given, happen to be solvents for the sulphonlic acid, but it is not essential that all of the solvents used be solvents for the sulphonlic acid.

Crude naphthalene sulphonlic acid is desirable because it not only works very satisfactorily, but is available at reasonable cost on the open market. In some instances, it may be preferred to

include a certain percentage of some such substance as carbon tetra-chloride to decrease the fire hazard of the mixture. In fact, five to fifteen per cent carbon tetra-chloride can be satisfactorily added to the above mixture.

In some cases, it may be exceptionally desirable to utilize a cleaning compound that is substantially non-inflammable. Such a mixture can be made by using—

|                                       | Per cent |
|---------------------------------------|----------|
| Crude naphthalene sulphonic acid..... | 6        |
| Carbon tetra-chloride.....            | 12       |
| Water.....                            | 29       |
| Alcohol.....                          | 53       |

15 To treat the metal in accordance with the present invention, it is first freed from mechanical dirt and excess grease. My cleaning mixture is then applied to the surface of the metal, and it is of considerable importance that this improved cleaner can be applied by spraying. The resulting fumes from spraying this cleaning solution are not objectionable as are the corrosive acid fumes that would result from the spraying of cleaning solutions containing mineral acids.

20 Another very important feature of the present invention resides in the fact that while with the prior art cleaners, it is essential that the cleaner be removed before painting, with the present cleaner it is not at all necessary to remove the same before painting, and in many instances there is a decided advantage to be gained by leaving the film formed by the cleaning spray upon the metal and to apply the paint, lacquer, or other coating directly upon the said film. As a matter of fact, the cleaning solution formed with the organic sulphonic acid and combination of solvents forms a desirable base for paints and lacquers, and in some classes of work, the presence of the film formed from the application of the cleaning fluid may take the place of the customary primer coat.

25 It will, of course, be appreciated that to enable the satisfactory deposition of the paint directly to the film of cleaning fluid, there be no excessive mechanical dirt or grease upon the sur-

face of said cleaning film. In the event that foreign matter should become deposited upon the cleaning film and that this cannot be removed by blasts of air, the coated metal can be washed, preferably with a solvent that will not entirely remove the cleaning film. Alcohol or benzene, either alone or mixed, can be used for this purpose, and while water might be used, it is preferred that no water be applied to the metal after the cleaning solution has been applied. Such solvents as those mentioned will not entirely remove, insofar as I have been able to ascertain, the film of cleaning material on the metal.

10 It is believed that the many advantages of my improved cleaning process over the prior art are apparent.

I claim:

1. A cleaning compound for metal surfaces such as iron or steel, comprising an organic sulphonic acid, water, and a solvent for grease, said compound being substantially devoid of mineral acid and the salts thereof.

2. A cleaning compound for metal surfaces such as iron or steel, comprising an organic sulphonic acid, water, a solvent for grease, and carbon tetra-chloride said compound being substantially devoid of mineral acid and the salts thereof.

3. A cleaning compound for metal surfaces such as iron or steel, comprising an organic sulphonic acid, water, and alcohol said compound being substantially devoid of mineral acid and the salts thereof.

4. A cleaning compound for metal surfaces such as iron or steel, comprising an organic sulphonic acid, water, alcohol, and benzene said compound being substantially devoid of mineral acid and the salts thereof.

5. A cleaning compound for metal surfaces such as iron or steel, comprising naphthalene, sulphonic acid, water, and a solvent for grease said compound being substantially devoid of mineral acid and the salts thereof.

45 MICHAEL W. FREEMAN. 45